

## UNITED STATES PATENT OFFICE

RALPH J. WIRSHING AND HENRY R. FAAS, OF DETROIT, MICHIGAN, ASSIGNORS TO  
GENERAL MOTORS RESEARCH CORPORATION, OF DETROIT, MICHIGAN, A CORPORA-  
TION OF DELAWARE

## ELECTROPLATING PROCESS

No Drawing.

Application filed January 10, 1927. Serial No. 160,310.

The invention relates to electroplating and has particular reference to the electrodeposition of nickel and chromium. It has been customary to deposit chromium upon nickel in order to produce a combined coating of high protective efficiency. Upon nickel deposits as hitherto produced, however, it has been difficult to apply a chromium deposit of more than a very limited thickness without causing the combined coating to peel off or loosen from the metal body beneath. In fact, when nickel is deposited by the usual methods of plating that metal, a subsequent application of chromium plating has been limited practically to that obtainable in about five minutes' plating.

We have found, however, that by use of a hot plating bath for deposition of the nickel a much softer and a much more adherent coating of nickel may be obtained. The softer deposit materially facilitates the operation of buffing, and the greater adhesion of the nickel layer enables a greatly increased thickness of chromium to be applied.

In the attempt to use the usual nickel sulphate bath at the elevated temperature at which we prefer to operate it is found that pitting of the nickel deposit occurs. The discovery has been made, however, that a bath containing nickel acetate is capable of depositing nickel at a much higher temperature than a nickel sulphate bath without the occurrence of pitting. In fact, the use of a low temperature with a nickel acetate bath seems to promote pitting whereas the high temperature operation inhibits pitting. Furthermore, the use of the nickel acetate bath at a high temperature enables a much higher current density to be used than has been found practicable with nickel sulphate baths thus facilitating a material increase in the rate of deposit of the metal.

In practice we have found that 200 grams nickel acetate, and 15 grams sodium chloride, per liter of water will provide a satisfactory bath. It will be understood, of course, that a considerable range of proportions is possible, for example, the sodium chloride may vary from 5-15 grams without materially affecting the results.

The nickel acetate may be added to the bath directly or it may be produced in the bath, as, for example, by reaction between acetic acid and nickel carbonate or basic carbonate.

The temperatures employed vary over a considerable range but should be above approximately 100° F. and the preferred range may be given as between 140 and 160° F.

The current density may be made quite high compared with that usual with other nickel baths. Best results have been obtained with densities of 15 to 100 amperes per square foot at the cathode although densities as high as 500 amperes per sq. ft. have given good results. Nickel anodes are used.

In the plating of nickel or ferrous metals it is customary to first coat the base metal with copper. When this procedure is followed we have found it preferable to plate the copper from a copper cyanide bath, thereby decreasing the occurrence of rust stimulating salts in the coating. It has been found desirable also to deposit the copper from a hot solution, good results having been obtained with the temperature of the copper bath maintained above 150° F.

When it is desired to deposit chromium on the nickel, a chromium plating bath of ordinary character may be used, for example, that of the type known as Sargent's solution, or a bath containing approximately 200 grams of chromic acid and 3 grams chromium sulphate per liter.

Proceeding as described above, we have found that thick deposits of chromium may be easily applied over nickel and that these deposits are very smooth and brilliant and the coating adheres strongly to the base metal.

Modifications may, of course, be made by those skilled in the art without departing from the invention and therefore we do not wish to be restricted to the details herein set forth except as required by the language of the appended claims in view of the prior art.

We claim:

1. The process of electrolytically depositing nickel comprising passing an electric current through a bath containing as its principal solute nickel acetate and including the

65

70

75

80

85

90

95

100

maintenance of the bath during electrodeposition at a temperature between the approximate limits of 100° to 160° F.

2. The process of electrolytically depositing nickel comprising passing an electric current through a bath containing as its principal solute nickel acetate, including the maintenance of the bath at a temperature of approximately 140° to 160° F.

10 3. The process as set forth in claim 2 including the use of a current density at the cathode of 15 to 100 amperes per square foot.

In testimony whereof we affix our signatures.

15

RALPH J. WIRSHING.  
HENRY R. FAAS.

20

25

30

35

40

45

50

55

60

65